

## 1

2,819,982

### PRODUCTION OF SILVER MIRRORS BY VOLATILISATION

Willem Westerveld, Jan Willem Van Tyen and Bartholomeus Haes, Eindhoven, Netherlands, assignors, by mesne assignments, to North American Philips Company, Inc., New York, N. Y., a corporation of Delaware

No Drawing. Application October 29, 1953  
Serial No. 389,156

Claims priority, application Netherlands  
November 15, 1952

3 Claims. (Cl. 117—35)

It has been suggested before to provide a method of producing silver mirrors by silver-coating and rendering incandescent a filament made of a metal having a very high melting point, such as tungsten or molybdenum. The article required to be coated with silver is then placed near the filament.

This method permits of providing, for example, glass bulbs for electric incandescent lamps or bowls for reflectors with a reflecting surface.

A known limitation consists in that silver wets the filament poorly and contracts in drops so that the silver drops from the wire. It was suggested before to add to the filament or to the silver a third metal apt to improve the adherence of the silver and to cause it to flow out about the filament. It was suggested to use as the flux the metals of the eighth group and more particularly platinum, palladium, iridium, rhodium, iron, nickel and cobalt and also beryllium.

Even the use of these metals gives rise to difficulties. It is true that precious metals, such as platinum have the desired effect, but the percentage to be added to the silver is comparatively high. The best results are obtained with a silver alloy containing from 5 to 15% of these metals. However, such alloys are far more expensive than the silver itself. Of the other metals a quantity of the order of 1% is added to the silver. The adherence of such alloys is comparatively poor and it may be necessary previously to coat the filament entirely with such an alloy by galvanic means.

According to the invention the flux used is silicon and this has the advantage that minute quantities, in the order

## 2

of 0.1%, are sufficient, the wetting of the filament being quite satisfactory. In addition, silicon satisfies the requirement that on volatilisation it does not bring about any change in colour of the silver mirror.

- 5 For carrying out the method according to the invention pieces of a silver alloy containing for example 0.1% silicon may be introduced into a filament of tungsten, molybdenum or similar high melting point metal. When glowing this alloy will spread quite evenly throughout 10 the surface of the filament.
- What is claimed is:
1. A method of producing silver mirrors comprising the steps, introducing an alloy of silver and a minute amount of silicon into a metallic filament consisting essentially of a refractory metal having a high melting point, and heating to incandescence said filament to evaporate the silver therefrom and deposit said silver on the surface of a body placed in the vicinity of said filament thereby to form a silver mirror on said body.
  2. A method of producing silver mirrors comprising the steps, introducing an alloy of silver and about 0.1% of silicon into a metallic filament consisting essentially of a refractory metal having a high melting point, and heating to incandescence said filament to evaporate the silver therefrom and deposit said silver on the surface of a body placed in the vicinity of said filament thereby to form a silver mirror on said body.
  3. A method of producing silver mirrors comprising the steps, introducing an alloy of silver and about 0.1% of silicon into a metallic filament consisting essentially of a refractory metal selected from the group consisting of tungsten and molybdenum, and heating to incandescence said filament to evaporate the silver therefrom and deposit said silver on the surface of a body placed in the vicinity of said filament thereby to form a silver mirror on said body.

### References Cited in the file of this patent

#### UNITED STATES PATENTS

|    |           |                |                |
|----|-----------|----------------|----------------|
| 40 | 2,079,784 | Williams       | May 11, 1937   |
|    | 2,138,637 | Leach          | Nov. 29, 1938  |
|    | 2,386,876 | Ogle et al.    | Oct. 16, 1945  |
|    | 2,424,085 | Bergsteinsson  | July 15, 1947  |
| 45 | 2,450,340 | Hensel et al.  | Sept. 28, 1948 |
|    | 2,450,850 | Colbert et al. | Oct. 5, 1948   |
|    | 2,450,856 | Colbert et al. | Oct. 5, 1948   |